

## UNITED STATES PATENT OFFICE

2,216,137

DIAZOTYPE PHOTOGRAPHIC PRINTING  
PAPER

Maximilian Paul Schmidt and Oskar Süs, Wiesbaden-Biebrich, Germany, assignors to Kalle & Co. Aktiengesellschaft, Wiesbaden-Biebrich, Germany

No Drawing. Application October 10, 1936, Serial No. 105,088. In Germany October 12, 1935

4 Claims. (Cl. 95—6)

The present invention relates to diazotype photographic printing papers.

It is known to manufacture light sensitive diazotype photographic printing papers which contain in the layer the two dyestuff components, namely the diazo compound and the azo component, serving for the production of the picture or the like. Papers of this kind only require for their development a treatment with alkalis, for example ammonia or soda solution. It has also been proposed to apply the alkali serving for the development alone or in admixture with an azo component on papers sensitized with diazo compounds before the exposure, the said alkali and/or azo component being applied in powder form. Papers of this kind can be developed by a simple treatment with water or steam respectively. They possess, however, only very poor keeping qualities. Moreover, they have the disadvantage that when in use they easily become dusty, i. e. give off fine particles of the alkali and/or the azo component, which gives rise to considerable inconvenience to the operator carrying out the work of printing.

One object of the present invention is the production of light sensitive materials to be developed by treatment with water which materials have better keeping qualities than the known materials of this kind. Another object of the invention is the production of light sensitive materials of the mentioned type which do not tend to give off fine particles of the substances which have been applied in powder form.

According to the invention, light sensitive diazotype materials are provided which contain as developing means a coupling component and a neutral salt of a weak base with a weak acid which latter is fugitive with steam, i. e. can be volatilized by means of steam below its normal boiling point. Such salts are the acetates and formates of zinc, cadmium and lead.

It is supposed that during the development of the new diazotype layers with steam, oxides or basic salts are formed from the said acetates or formates respectively with the elimination of the hydrolytically separated acids whereby the diminution of the acidity of the layers necessary for the coupling process is obtained.

As diazo compounds advantageously such which couple rapidly, i. e. couple under neutral or acid conditions are used.

We have discovered that the said light sensitive materials in which either the said neutral salt or the coupling component or both have been applied to the support in powder form, for ex-

ample by rubbing the powder in, can be obtained practically free from dust by treating them after the application of the constituents, with a strong current of air, for example by blowing the air on to them or by sucking it off from them. The power of the current of air may amount to some atmospheres. In place of air other inert gases may be employed. It is a surprising fact that during this treatment a sufficient quantity of the developing substances and the azo components, when they have been applied by rubbing them into the paper, remains behind to enable complete development still to be effected, whilst, on the other hand, inconvenience in the working operations is avoided. For further preventing a slight development of dust when employing papers of the aforesaid kind they may, after the above described treatment, be further treated with rollers, whereby a better closure of the surface of the paper and consequently a better adherence of the powdered substances is obtained.

The following examples illustrate the invention:

(1) Paper sensitized with a solution of 36 grams of the zinc chloride salt of the diazo compound of 2' 6"—dichlorobenzyl-4-amino-1-aniline and 30 grams of citric acid has rubbed into it a powder consisting of 125 grams of phloroglucine and 250 grams of calcium acetate. After the rubbing in operation loose powder remaining on the surface of the paper is removed by blowing dry air under pressure on to the latter. By subsequent calendering an increase of the power of adherence of the powder which still remains is obtained. Paper subsequently treated in this way after the rubbing in of the powder, in contradistinction to paper which has not been so treated, no longer becomes dusty, i. e. yields up dust. The speed of development and the intensity are retained in their entirety.

(2) Paper is sensitized with a solution containing 90 grams of the diazo compound of 1-amino-4-benzoylamino-2,5-diethoxybenzene, 45 grams of citric acid and 3 litres of water and has rubbed into it by mechanical means an intimately mixed powder consisting of 125 grams of phloroglucine and 250 grams of zinc acetate. If desired, both in this case and in Example 1, inert substances, such as starch, may be added for diluting the powder. The after-treatment of the paper is carried out as described in Example 1. In place of the zinc acetate also the corresponding formic acid salt may be employed.

(3) The sensitization of the paper is effected

as in Example 1. The powder applied by rubbing it in has the following composition:

|                 | Grams |
|-----------------|-------|
| 5 Phloroglucine | 125   |
| Lead acetate    | 318   |

The after-treatment of the paper is carried out as in Example 1.

(4) The sensitization of paper is effected as 10 in Example 2. The developing powder, which is applied by rubbing it in, consists of:

|                                 | Grams |
|---------------------------------|-------|
| 15 Phloroglucine                | 60    |
| Cadmium acetate                 | 200   |
| Glauber's salt (sodium sulfate) | 120   |

The after-treatment of the paper is carried out as in Example 1.

(5) Paper is sensitized with a solution containing 15 grams of the diazo compound of 1-phenylthioacetylaminio-2,5-dimethoxy-4-amino-benzene, 5 grams of citric acid, 5 grams of boric acid, 5 grams of aluminium sulphate and 1 litre of water and has rubbed into it a mixture of 60 20 grams of phloroglucine, 200 grams of cadmium acetate and 120 grams of Glauber's salt. The

after-treatment is carried out as in Example 1.

We claim:

1. A light-sensitive material which comprises a diazo compound and developing means which comprise a coupling component and a neutral 5 reacting salt of a weak base with a weak acid selected from the group consisting of the acetates and formates of lead, zinc, and cadmium, the material being free from dust.

2. A light-sensitive material which comprises 10 a diazo compound and developing means which comprise a coupling component and zinc formate, the material being free from dust.

3. A light-sensitive material which comprises 15 a rapidly coupling diazo compound and developing means which comprise a coupling component and a neutral reacting salt of a weak base with a weak acid selected from the group consisting of the acetates and formates of lead, zinc, and cadmium, the material being free from dust. 20

4. A light-sensitive material which comprises a diazo compound and developing means which comprise a coupling component and zinc acetate, the material being free from dust. 25

MAXIMILIAN PAUL SCHMIDT. 25  
OSKAR SÜS.